

F. J. LYSER.

CONCENTRATION OF ORES.

APPLICATION FILED JULY 8, 1916.

1,203,374.

Patented Oct. 31, 1916

2 SHEETS—SHEET 1.



Fig. 1.

Inventor:  
Flerry James Lyster  
By Henry B. Williams  
Attorney

F. J. Lyster.

### CONCENTRATION OF ORES.

APPLICATION FILED JULY 8, 1916.

1,203,374.

Patented Oct. 31, 1916.

2 SHEETS—SHEET 2

Fig. 2.



Fig. 3.

*Inventor:*

Henry James Lyder  
By Henry H. Willard  
Attorney.

# UNITED STATES PATENT OFFICE.

FLEURY JAMES LYSTER, OF BROKEN HILL, NEW SOUTH WALES, AUSTRALIA, ASSIGNOR,  
BY MESNE ASSIGNMENTS, TO MINERALS SEPARATION AMERICAN SYNDICATE (1913)  
LIMITED, OF LONDON, ENGLAND.

## CONCENTRATION OF ORES.

1,203,374.

Specification of Letters Patent. Patented Oct. 31, 1916.

Original application filed May 8, 1913, Serial No. 766,346. Divided and this application filed July 8, 1916.  
Serial No. 108,208.

To all whom it may concern:

Be it known that I, FLEURY JAMES LYSTER, subject of the King of Great Britain and Ireland, and residing at Broken Hill, in 5 the State of New South Wales, Commonwealth of Australia, have invented certain new and useful Improvements in the Concentration of Ores, of which the following is a specification, reference being had therein 10 to the accompanying drawings, forming part thereof.

This invention relates to improvements in the concentration of ores and is particularly applicable to the separation of mixed zinc 15 and lead sulfid ores, and this application is a division of my application filed May 8, 1913, Serial No. 766,346.

The object of this invention is to separate metalliferous portions of an ore such, for 20 example, as the sulfid of lead (galena) from other portions of the ore, and more particularly to effect a differential or selective flotation in the treatment of mixed zinc and lead sulfid ores, to wit: the separation 25 of lead sulfid (galena) from zinc sulfid (blende), obtaining a product relatively rich in lead on the one hand, and a zinc product relatively low in lead on the other hand.

I have discovered that sulfid of lead 30 (galena) may be separated from sulfid of zinc (blende) by subjecting the ore or metalliferous materials to a flotation-separation treatment at a low temperature with eucalyptus oil or other frothing agent and with 35 agitation or aeration in a neutral or alkaline solution of the chlorid of a metal such as sodium chlorid and that alkalinity produced in said solution by an alkaline hydrate in some instances promotes the separation.

40 The suitability of any given substance in a neutral or alkaline solution can be easily determined by a laboratory test as herein-after described.

In carrying this process into effect a plant 45 similar to that employed in and common to agitation froth processes may be employed. I have shown in the accompanying drawings two forms of apparatus adapted for carrying out my process.

50 Figure 1 is a longitudinal elevation and Fig. 2 a cross-section of a unit with the supply devices in elevation, and Fig. 3 is a sec-

tional elevation of an apparatus suitable for testing.

I will now describe my process as carried 55 out in the apparatus shown in Figs. 1 and 2.

The ore is first ground to a suitable degree of fineness (preferably to slimes so that the different metallic sulfid particles are disassociated from each other). This finely 60 ground ore with its accompanying circuit water (which is a solution such as herein-before described) is led into a settler or thickener A to remove excess water. The thickened pulp is then led into a vessel B, 65 from which it passes to the first centrifugal pump C<sup>1</sup> of the series C<sup>1</sup>, C<sup>2</sup>, C<sup>3</sup>, C<sup>4</sup>, C<sup>5</sup>, C<sup>6</sup>. These centrifugal pumps are each connected to the individual members of a corresponding series of separating boxes D<sup>1</sup>, D<sup>2</sup>, D<sup>3</sup>, D<sup>4</sup>, 70 D<sup>5</sup>, D<sup>6</sup>. These centrifugal pumps act as agitators or mixers and means are provided (such as an inlet pipe E) for feeding in the requisite amount of eucalyptus oil or other frothing agent, about 2 lbs. per ton of material treated, as well as the requisite amount 75 of air (such as by a tap F) into the suction pipe G<sup>1</sup> thereof, which is connected to the feed vessel B. The centrifugal pump C<sup>1</sup> draws in pulp, air, and frothing agent, and 80 produces an intimate mixture which is discharged through the outlet pipe H to the separator box D<sup>1</sup>, the delivery of the pump being controlled by the admission of air by the tap F. The particles of lead sulfid 85 (galena) are found to rise to the top of the separator box D<sup>1</sup>, where an inverted pyramid J<sup>1</sup> diverts the froth toward the discharge lip or launder K<sup>1</sup>, from which it flows to the receptacle for settling and collecting the lead concentrate. The particles which do not rise or float, together with the balance of the water, sink to the bottom of the box D<sup>1</sup> and are there withdrawn by the outlet pipe L<sup>1</sup> which is connected to the suc-

tion pipe G<sup>2</sup> of the next pump C<sup>2</sup> of the series, and the operation is repeated, the residues of the separator box D<sup>2</sup> passing to the centrifugal pump C<sup>3</sup> of the next in series. In the plant illustrated in the accompanying drawings there are six separator boxes and their attendant pumps, which comprise one series or unit, but it will be understood that this number is de-

pendent upon the proportion of mineral contained in the ore and the degree of agitation and aeration required, the repetition of the operations being carried on until the grade of the concentrates becomes too low in lead and the zinc begins to appear therein. The temperature I prefer is below 100° Fah. That is to say, the operation is conducted at the ordinary temperature and no extraneous heat is utilized.

I have observed in working the process for the selective flotation of lead sulfids from what are known as calcitic slimes at Broken Hill that an excessive alkalinity tends to retard the selective flotation of the lead sulfid particles. Therefore, when the process is used with this ore for this purpose with an alkaline solution, the solution should be only slightly alkaline but sufficient to respond to the well known methyl orange test.

The suitability of the substances hereinbefore indicated and the proportion thereof to the solution and the degree and duration of agitation or aeration of the material treated can be determined in a laboratory test which may be conducted as follows in an apparatus such as is illustrated in Fig. 3 of the accompanying drawings. This apparatus comprises an agitating or mixing vessel N having a rotating impeller O, a separating box P on the side thereof connected to the mixer by a passage R and by a flexible hose pipe S at the bottom. In carrying out a test the mixing vessel N contains the solution which corresponds with the circuit water of the working plant, and eucalyptus or other frothing agent is then added in measured quantities. The impeller O is then rotated at about 1700 revolutions per minute and a charge of about 448 grams of ore is fed in. Sufficient solution is added to fill the separating box P to the level of its discharge lip. The agitated pulp is forced through the passage R into the separating box P and the float or froth rising to the surface is skimmed off over the lip. The pulp is continuously circulated by being drawn from the bottom of the box P by the pipe S back into the mixer N by the action of the impeller O. The flotation is continued until the float or froth is noticed by observation to become lower in lead and the zinc begins to appear therein. The appearance of the concentrate being skimmed off over to the lip of the separating box will indicate the duration of agitation necessary to obtain a good concentrate combined with a good recovery, while experience will indicate the amount of frothing agent necessary, and further quantities may be added at intervals as found necessary. The residue is run off from the bottom of the machine by disconnecting the flexible hose of pipe S. Repeated trials with different solutions

and with different strengths will indicate what is best suited to the particular ore under treatment. The ascertained duration of agitation and aeration will govern the number of separator boxes which will be necessary in the working plant when that hereinbefore described is used.

The following are examples of solutions which have been used by me in obtaining a selective separation of the lead sulfids from the zinc sulfids in the ore heretofore referred to, known as calcitic slimes at Broken Hill, to which my process is peculiarly well suited, averaging about eleven (11%) per cent. of zinc and about thirteen (13%) per cent. of lead, using about from two (2) to five (5) lbs. of eucalyptus oil per ton.

|                     |     |                    |
|---------------------|-----|--------------------|
| Sodium chlorid      | 800 | grains per gallon. |
| { Sodium chlorid    | 800 | grains " "         |
| with                |     |                    |
| Calcium hydrate     | 1.8 | " "                |
| Sodium chlorid      | 800 | " "                |
| with                |     |                    |
| Calcium hydrate     | 3.6 | " "                |
| Sodium chlorid      | 800 | " "                |
| with                |     |                    |
| Calcium hydrate     | 18  | " "                |
| Potassium chlorid   | 800 | " "                |
| { Potassium chlorid | 800 | " "                |
| with                |     |                    |
| Calcium hydrate     | 1.8 | " "                |
| Potassium chlorid   | 800 | " "                |
| with                |     |                    |
| Calcium hydrate     | 3.6 | " "                |
| Potassium chlorid   | 800 | " "                |
| with                |     |                    |
| Calcium hydrate     | 18  | " "                |
| Calcium chlorid     | 300 | " "                |
| { Calcium chlorid   | 300 | " "                |
| with                |     |                    |
| Calcium hydrate     | 1.8 | " "                |
| Calcium chlorid     | 300 | " "                |
| with                |     |                    |
| Calcium hydrate     | 3.6 | " "                |
| Barium chlorid      | 300 | " "                |
| { Barium chlorid    | 300 | " "                |
| with                |     |                    |
| Calcium hydrate     | 1.8 | " "                |
| Barium chlorid      | 300 | " "                |
| with                |     |                    |
| Calcium hydrate     | 3.6 | " "                |
| Magnesium chlorid   | 300 | " "                |
| { Magnesium chlorid | 300 | " "                |
| with                |     |                    |
| Calcium hydrate     | 1.8 | " "                |
| Magnesium chlorid   | 300 | " "                |
| with                |     |                    |
| Calcium hydrate     | 3.6 | " "                |

85

96

95

100

105

110

115

125

130

I have further discovered that the residues obtained as before described containing the bulk of the zinc sulfids may be further treated by flotation separation to produce a concentrate rich in zinc by first dewatering and thickening the pulp and then submitting it to a repetition of the flotation separation, using, however, sufficient water in lieu of the solution previously employed, or by further continuing the process hereinbefore described, after the recovery of the lead sulfids (galena) in a separate dezincing unit until the zinc sulfids (blende) appear upon the surface of the solution and are carried over into the launder hereinbefore mentioned. In operation I prefer the former to the latter method for the recovery of the zinc sulfids (blende). In this way a zinc concentrate may be obtained and thereby both the lead sulfids and zinc

sulfids recovered in separate products by flotation separation without recourse to separation by gravitation or tables or vanners as heretofore.

5 I claim:

1. A process of concentrating ores which consists in agitating and aerating an ore pulp containing in solution a chlorid of a metal in quantity sufficient to substantially facilitate the formation of a froth of concentrates, and separating the froth.

10 2. A process of concentrating ores which consists in agitating and aerating an ore pulp containing a small proportion of a frothing agent and containing in solution a chlorid of a metal in quantity sufficient to substantially facilitate the formation of a froth of concentrates, and separating the froth.

15 3. A process of concentrating ores which consists in agitating and aerating an ore pulp containing in solution an alkaline hydrate and a chlorid of a metal in quantity sufficient to substantially facilitate the formation of a froth of concentrates, and separating the froth.

20 4. A process of concentrating ores which consists in agitating and aerating an ore pulp containing a small proportion of a frothing agent and containing in solution an alkaline hydrate and a chlorid of a metal in quantity sufficient to substantially facilitate the formation of a froth of concentrates, and separating the froth.

25 5. A process of concentrating ores which consists in agitating and aerating an ore pulp containing sodium chlorid in solution in quantity sufficient to substantially facilitate the formation of a froth of concentrates, and separating the froth.

30 6. A process of concentrating ores which consists in agitating and aerating an ore pulp containing a small proportion of a frothing agent and containing sodium chlorid in solution in quantity sufficient to substantially facilitate the formation of a froth of concentrates, and separating the froth.

35 7. A process of concentrating ores which consists in agitating and aerating an ore pulp containing in solution an alkaline hydrate and sodium chlorid in quantity sufficient to substantially facilitate the formation of a froth of concentrates, and separating the froth.

40 8. A process of concentrating ores which consists in agitating and aerating an ore pulp containing a small proportion of a frothing agent and containing in solution an alkaline hydrate and sodium chlorid in quantity sufficient to substantially facilitate the formation of a froth of concentrates, and separating the froth.

45 9. A process of concentrating ores which consists in agitating and aerating an ore

pulp containing in solution calcium hydrate and a chlorid of a metal in quantity sufficient to substantially facilitate the formation of a froth of concentrates, and separating the froth.

50 10. A process of concentrating ores which consists in agitating and aerating an ore pulp containing a small proportion of a frothing agent and containing in solution calcium hydrate and a chlorid of a metal in quantity sufficient to substantially facilitate the formation of a froth of concentrates, and separating the froth.

55 11. A process of concentrating ores which consists in agitating and aerating an ore pulp containing in solution calcium hydrate and sodium chlorid in quantity sufficient to substantially facilitate the formation of a froth of concentrates, and separating the froth.

60 12. A process of concentrating ores which consists in agitating and aerating an ore pulp containing a small proportion of a frothing agent and containing in solution calcium hydrate and sodium chlorid in quantity sufficient to substantially facilitate the formation of a froth of concentrates, and separating the froth.

65 13. A process for the separation of lead sulfids from zinc sulfids in an ore containing mixed lead and zinc sulfids which consists in subjecting such an ore to the agitation froth process by agitation in a pulp containing in solution a chlorid of a metal in quantity sufficient to substantially facilitate the formation of a froth of concentrates wherein the lead sulfids predominate.

70 14. A process for the separation of lead sulfids from zinc sulfids in an ore containing mixed lead and zinc sulfids which consists in subjecting such an ore to the agitation froth process by agitation in a pulp containing a small proportion of a frothing agent and containing in solution a chlorid of a metal in quantity sufficient to substantially facilitate the formation of a froth of concentrates wherein the lead sulfids predominate.

75 15. A process for the separation of lead sulfids from zinc sulfids in an ore containing mixed lead and zinc sulfids which consists in subjecting such an ore to the agitation froth process by agitation in a pulp containing in solution an alkaline hydrate and a chlorid of a metal in quantity sufficient to substantially facilitate the formation of a froth of concentrates wherein the lead sulfids predominate.

80 16. A process for the separation of lead sulfids from zinc sulfids in an ore containing mixed lead and zinc sulfids which consists in subjecting such an ore to the agitation froth process by agitation in a pulp containing a small proportion of a frothing agent and containing in solution an alkaline hy-

70

75

80

85

90

95

100

105

110

115

120

125

130

drate and a chlorid of a metal in quantity sufficient to substantially facilitate the formation of a froth of concentrates wherein the lead sulfids predominate.

5 17. A process for the separation of lead sulfids from zinc sulfids in an ore containing mixed lead and zinc sulfids which consists in subjecting such an ore to the agitation froth process by agitation in a pulp 10 containing sodium chlorid in solution in quantity sufficient to substantially facilitate the formation of a froth of concentrates wherein the lead sulfids predominate.

15 18. A process for the separation of lead sulfids from zinc sulfids in an ore containing mixed lead and zinc sulfids which consists in subjecting such an ore to the agitation froth process by agitation in a pulp containing a small proportion of a frothing 20 agent and containing sodium chlorid in solution in quantity sufficient to substantially facilitate the formation of a froth of concentrates wherein the lead sulfids predominate.

25 19. A process for the separation of lead sulfids from zinc sulfids in an ore containing mixed lead and zinc sulfids which consists in subjecting such an ore to the agitation froth process by agitation in a pulp 30 containing in solution an alkaline hydrate and sodium chlorid in quantity sufficient to substantially facilitate the formation of a froth of concentrates wherein the lead sulfids predominate.

35 20. A process for the separation of lead sulfids from zinc sulfids in an ore containing mixed lead and zinc sulfids which consists in subjecting such an ore to the agitation froth process by agitation in a pulp 40 containing a small proportion of a frothing agent and containing in solution an alkaline hydrate and sodium chlorid in quantity sufficient to substantially facilitate the formation of a froth of concentrates wherein the lead sulfids predominate.

45 21. A process for the separation of lead sulfids from zinc sulfids in an ore contain-

ing mixed lead and zinc sulfids which consists in subjecting such an ore to the agitation froth process by agitation in a pulp 50 containing in solution calcium hydrate and a chlorid of a metal in quantity sufficient to substantially facilitate the formation of a froth of concentrates wherein the lead sulfids predominate.

55 22. A process for the separation of lead sulfids from zinc sulfids in an ore containing mixed lead and zinc sulfids which consists in subjecting such an ore to the agitation froth process by agitation in a pulp 60 containing a small proportion of a frothing agent and containing in solution calcium hydrate and a chlorid of a metal in quantity sufficient to substantially facilitate the formation of a froth of concentrates wherein 65 the lead sulfids predominate.

70 23. A process for the separation of lead sulfids from zinc sulfids in an ore containing mixed lead and zinc sulfids which consists in subjecting such an ore to the agitation froth process by agitation in a pulp containing in solution calcium hydrate and sodium chlorid in quantity sufficient to substantially facilitate the formation of a froth 75 of concentrates wherein the lead sulfids predominate.

80 24. A process for the separation of lead sulfids from zinc sulfids in an ore containing mixed lead and zinc sulfids which consists in subjecting such an ore to the agitation froth process by agitation in a pulp containing a small proportion of a frothing agent and containing in solution calcium hydrate and sodium chlorid in quantity sufficient to substantially facilitate the formation 85 of a froth of concentrates wherein the lead sulfids predominate.

In testimony whereof I have affixed my signature.

FLEURY JAMES LYSTER.

Witnesses:

ARTHUR GORE COLLISON,  
FLORENCE MANTHORPE.